

Aug. 28, 1928.

J. V. MARSHALL

1,681,943

LADLE LINING

Filed Dec. 18, 1925

*Fig. 1,*



*Fig. 2,*



*Fig. 3,*



*Fig. 5,*



*Fig. 4,*



*Fig. 6,*



*Fig. 7,*



Jas. V. Marshall  
INVENTOR  
BY  
John E. Bubbell  
ATTORNEY

## UNITED STATES PATENT OFFICE.

JAMES V. MARSHALL, OF NEW CASTLE, PENNSYLVANIA, ASSIGNOR TO NEW CASTLE REFRactories COMPANY, OF NEW CASTLE, PENNSYLVANIA, A CORPORATION OF DELAWARE.

## LADLE LINING.

Application filed December 18, 1925. Serial No. 76,185.

My present invention relates to ladles for handling molten metal, and particularly to the small or moderate sized ladles such as are commonly employed in iron, steel, and 5 brass foundries to receive molten metal from a melting furnace and to carry it to, and pour it into the molds in which the metal is cast.

The general object of the present invention is to provide improved linings for ladles 10 of the type referred to. Heretofore it has been the usual practice to line such ladles with fire clay daubed on the inner side of the ladle while the clay is in a moist plastic 15 condition. In accordance with the present invention, ladle linings are formed of parts of suitable refractory material which are shaped to fit the ladles to be lined and are hardened by being baked or fired before being put into the ladles in which they are to 20 be used.

The use of my improved ladle linings gives 25 important practical advantages over the common prior practice of lining ladles by daubing plastic fire clay on the inner walls of the ladle. For example, my improved linings may be made of less average thickness than the plastic fire clay lining thus giving increased ladle capacity. My im- 30 proved ladle linings are much more durable than plastic fire clay linings. Moreover, the improved linings may be put in place and renewed more quickly and easily than can plastic clay linings, and as soon as the im- 35 proved lining is put in place in a ladle the latter is ready for use, whereas a ladle lined with plastic clay cannot be put in use until the lining is thoroughly dried.

The various features of novelty which 40 characterize my invention are pointed out with particularity in the claims annexed to and forming a part of this specification. For a better understanding of the invention how- 45 ever, its advantages and specific objects at- tained with its use, reference should be had to the accompanying drawings and descrip- 50 tive matter in which I have illustrated and described preferred embodiments of my in- vention.

## 50 Of the drawings:

Fig. 1 is an elevation in section of a ladle and its linings;

Fig. 2 is a side elevation of the ladle lining shown in Fig. 1;

Fig. 3 is a plan view of a ladle lining of 55 modified form;

Fig. 4 is a section on the line 4—4 of Fig. 3;

Fig. 5 is a plan view of a ladle lining of a third form;

Fig. 6 is a section on the line 6—6 of Fig. 60 5; and

Fig. 7 is a vertical section of a ladle of still different form.

In Fig. 1 of the drawings I have shown a casting ladle A of conventional type lined 65 by a cup shaped body B of suitable refractory material baked or fired before insertion in the ladle and having its external surface shaped to fit snugly against the inner surface of the ladle. The ladle lining B has a 70 rounded bottom to fit against the saucer shaped bottom portion of the ladle A. When the bottom of the ladle to be lined is flat, the lining will have a flat bottom as does the ladle lining shown in Figs. 3 and 4. 75

Instead of forming the ladle lining in a single piece as shown in Fig. 1, it may well be formed in sections of different shapes. For example, as shown in Figs. 3 and 4, the ladle lining is formed by an integral disc 80 like bottom part b and curved stave portions b'. The ladle lining shown in Figs. 5 and 6, comprises a saucer shaped bottom portion b<sup>2</sup> and an upper portion formed by stave- 85 like parts b<sup>3</sup> relatively shorter than the parts b' of Figs. 3 and 4. The type of ladle lining shown in Fig. 7 comprises a saucer shaped bottom part b<sup>2</sup>, and an upper portion formed by one or more annular sections, two such sections being shown in Fig. 7. 90

While a one piece ladle lining as shown in Figs. 1 and 2 possesses the advantage of simplicity and maximum ease of installation and replacement, a ladle lining composed of a few simple sections as shown in 95 Figs. 4 to 7, possesses the practically desirable characteristics that the different sections are easy to make and install, and damaged sections may be replaced without the necessity for renewing undamaged sections. 100 Further local irregularities in form of the ladle or the lining are of less consequence with the sectional lining than with the one piece lining.

The joints between the different sections 105 may be plain butt joints as shown in Fig. 7, or they may be specially shaped to facilitate the sealing of the joints and to prevent the

sections from separating. For example, the sections may be shaped to form tongue and groove joints as shown in Fig. 3, or to provide interlocking joints as shown in Figs. 5 and 6. The joints may be sealed by means of a refractory cement or mortar of suitable composition. A saucer shaped bottom part of hardened refractory material such as the part  $b^2$  may sometimes be used to line the bottom portion of a ladle which has its upper portion lined with fire clay daubed on the corresponding portion of the ladle while in a plastic condition. A wide range of refractory materials such as fire clay and other refractory clays, magnesite, graphite, mica schist, chrome, silicon carbide, fused alumina, silica, dolomite, and fire sand are available for use in the construction of my improved ladle linings, the choice depending upon cost considerations, the temperature and nature of the molten metal handled, and other conditions of use.

While in accordance with the provisions of the statutes, I have illustrated and described the best form of embodiment of my invention now known to me, it will be apparent to those skilled in the art that changes may be made in the form of the apparatus disclosed without departing from the spirit

of my invention as set forth in the appended claims and that in some cases certain features of my invention may be used to advantage without a corresponding use of other features.

Having now described my invention what I claim as new and desire to secure by Letters Patent is:

1. A ladle lining comprising a cup-shaped body of hardened refractory material adapted to be inserted in and form a lining for a molten metal holding ladle.
2. A ladle lining comprising a bottom section and curved upper sections of hardened refractory material adapted to be assembled into a cup-like structure.
3. A ladle lining comprising an integral saucer shaped piece of hardened refractory material adapted to be inserted in and line the bottom portion of a molten metal holding ladle.
4. A cup-shaped ladle lining comprising an integral saucer shaped bottom section and a separate hollow upper section each formed of hardened refractory material.

Signed at New Castle, in the county of Lawrence, and State of Pennsylvania, this 14th day of December, A. D. 1925.

JAMES V. MARSHALL.